

Patented June 1, 1926.

## UNITED STATES PATENT OFFICE.

RONALD WILD, OF HOLMESFIELD, ENGLAND, ASSIGNOR, BY MESNE ASSIGNMENTS, TO  
RUSTLESS IRON CORPORATION OF AMERICA, A CORPORATION OF MARYLAND.

## MANUFACTURE OF FERROCHROMIUM ALLOY.

No Drawing.

Application filed February 5, 1923. Serial No. 617,171.

The present invention is for improvements in and relating to the manufacture of alloys of chromium and iron, such, for example, as ferro-chrome and metal of the type commonly known as stainless or unstainable iron and steel.

It is already known to submit molten crude ferro-chrome to an oxidizing blow with the object of obtaining an alloy of reduced content in impurities, such as carbon and silicon, which are removable by oxidation. In this operation, oxidation of the chromium takes place to a greater or lesser degree, and the loss of the metal in this way may be considerable. The present invention aims at providing an improved process of this kind whereby impurities of the aforesaid type may be eliminated, or brought down to the desired lower content, while loss of chromium through oxidation by the blow is reduced.

According to this invention, the manufacture of alloys of iron and chromium such, for instance, as ferro-chrome or stainless-iron or stainless-steel, by a process of the type wherein a crude basis metal comprising iron and chromium and containing impurities, such as carbon and silicon, removable by oxidation is subjected in the molten state to an oxidizing blow in order to reduce the content of said impurities, is characterized by the employment in the iron-chromium mixture or alloy submitted to the blow of an additional oxidizable element, that is to say, an element additional to the impurity or impurities to be removed, (such as carbon and silicon) and other than silicon, which element is more oxidizable than chromium at the temperature of the blowing operation, for the purpose of reducing the aforesaid loss of chromium during oxidation of the impurities.

The preferred additional oxidizable element is a metal which while more oxidizable than chromium is sufficiently less oxidizable than the impurities to be removed as not to be burnt away before the desired degree of purification of the alloy has been effected. For example, manganese may be added to the iron-chromium mixture or alloy to be blown, and such addition may be conveniently made in the form of ferro-manganese, or other suitable manganese-bearing alloy, in sufficient quantity to reduce to the

minimum possible the oxidation of the chromium during the subsequent blowing operation.

Alternatively, the element protective to the chromium may be introduced during the preparation of the basis metal to be blown by reducing a reducible compound of chromium in presence of iron (for instance, by reducing a reducible iron-chromium compound such as chromite) and of said protective element or of a reducible compound thereof. For instance, the reduction may be carried out in the presence of ferro-manganese, or of a reducible oxidized manganese compound.

According to the preferred mode of operation of this invention, the improved process for the manufacture of alloys of iron and chromium, such as ferro-chrome or stainless-iron or stainless-steel consists in first producing a crude basis metal of a nature specially favourable to purification with a blow by reducing a suitable reducible chromium compound in presence of iron (for instance, by reducing a reducible iron-chromium compound such as chromite) with substantially the chemical equivalent of a silicon-reducer (free from carbon or of such content therein as shall not be detrimental to the final alloy desired, for instance, low-carbon ferro-silicon) and then submitting the low-carbon-, high-silicon-basis metal so produced, after addition thereto of the requisite quantity of a protective element for the chromium for example, ferro-manganese, or the equivalent of another suitable manganese alloy, to desilicizing with an oxidizing blow.

Other conditions being alike, silicon is more conveniently eliminated than carbon by an oxidizing blast and as silicon-reducers, such, for instance, as ferro-silicon, of low carbon content may be obtained without difficulty, this preferred method of operation provides a means of economically obtaining a low-carbon purified product in a simple and practically direct manner. The type of basis metal produced by silicon reduction cannot be obtained directly from the blast furnace or the cupola, and the temperature at which the reduction takes place is also sufficient to enable the oxidation of the impurities in the crude alloy by an air blast to proceed without the necessity for the ad-

dition of a special reagent to raise the temperature for the blowing operation, but in the absence of a protective element of the type aforesaid the usual disadvantage is experienced of undue loss of chromium by oxidation.

Alternatively, the reduction with the silicon-reducer may be effected as aforesaid in presence of the element which will be protective to the chromium; or silico-manganese may be employed as reducer, in which case the reducing agent may itself provide the protective element required.

Stainless chrome-iron or chrome-steel may be directly prepared by effecting the reduction of the chromium-compound (preferably with a silicon reducer as aforesaid) within a bath of molten iron or steel substantially free from carbon, or of such content therein as shall provide for the desired proportion of carbon in the final alloy metal, said bath being proportioned so as to provide a basis metal for the blow of the metallic composition to yield as the purified product a stainless iron-chromium alloy metal. Or a ferro-chrome may be initially produced and then fused with the appropriate quantity of iron or steel, and the metal submitted to the blow. Or the ferro-chrome may be blown under the prescribed conditions prior to fusion with the iron or steel. In each case, the protective element may be introduced at any convenient stage prior to the blow, for example, during the preparation of the basis metal in the manner described.

The proportion of manganese to be utilized for the purpose of protecting the chromium in the basis metal submitted to the blow depends upon circumstances, such as the metallic composition of the basis alloy and the proportion of oxidizable impurities present therein. In the case of a crude basis metal of the metallic composition to yield as the purified product a stainless chrome-iron or chrome-steel, i. e. a metal of a chromium content substantially between 9 and 16 per cent, it may be said that the minimum proportion of manganese to protect the chromium is the quantity represented by approximately two-thirds of the proportion of the total oxidizable impurities, such as carbon and silicon and not substantially less than 2.5 per cent where said impurities are below 3.5 per cent. Iron-chromium alloys of a higher chromium content than that of stainless metal, for example, ferro-chrome do not behave analogously to the former metal in this respect, and in spite of the higher content in chromium the proportion of manganese relatively thereto may be comparatively small. With an increase in the carbon content of the fused metal, it may be found advisable to increase the proportion of manganese in the case both of metal of the composition of stainless-iron or stain-

less-steel and of iron-chromium alloys of a higher chromium content such as ferro-chrome.

The reduction mixture may be made up in the form of briquettes, which are then heated to the temperature necessary to start the reaction. The heat evolved by combination of the oxides and the silicon-reducer enables the operation then to proceed with the minimum application of external heat. Suitable fluxes, such as lime and fluorspar, may be employed to facilitate the reaction. The reduction with ferro-silicon is preferably effected in presence of a reagent, such as limestone or lime, which is capable of combining with the oxidized silicon and forming a slag therewith.

A ferro-silicon of high silicon content, for example, 80 to 90 per cent, of silicon, is the preferred form of this reagent, as thereby a more energetic reaction is brought about, and a product of higher content in the metal or metals other than the iron is obtained.

The reduction may be carried out in any suitable furnace in which the necessary high temperature is attainable, and it has been found convenient to use an electric furnace, for instance, of the Snyder or Heroult type. For small-bulk charges, an ordinary crucible furnace may be employed. External heating may be applied in order to maintain the necessary high temperature throughout the reduction. Like considerations as to the maintenance of requisite high temperature conditions apply to the blowing operation.

I have found that a generally convenient method of carrying the invention into effect is to fuse the ferro-silicon or other silicon-reducer with a part of the charge of the slag-forming reagent, such as limestone, either alone or in presence of a bath of iron or steel, and then to add the reducible charge to the melt, preferably in successive quantities, the metallurgical reaction being assisted by agitation of the bath by rabbling, and by the addition of the remainder of the slag-forming reagent as required.

When the ebullition produced in the bath by the reducing action has subsided, and providing the element protective to the chromium has not already been introduced during the reduction, the addition of this element is now made. For instance, ferro-manganese may be added to the bath, and when the whole mass has been brought to a state of fusion, the iron-chromium alloy, containing silicon, carbon and manganese, is submitted to the oxidizing blow.

A convenient and economical way of delivering the air blast into the molten metal is by means of a wrought-iron pipe, covered with fireclay sleeves, and jointed with fireclay. This pipe may lead into the furnace directly on to the hearth thereof.

The blow may be a blast of cold or pre-heated air under a forced or suction draught. For the purpose of curtailing the period of the blow, or, at any convenient stage of the process, to assist in the oxidation of the impurities in the metal, the blast may advantageously be caused to carry chromite, or other reducible oxidized compound of chromium, or a base such as lime, in a finely pulverized state, into the molten mass.

The following are descriptions by way of example of the application of the invention to the manufacture respectively of a high-chromium ferro-chrome, and of stain-less metal, of low content both in carbon and silicon.

*Example I.*

A charge of 54 lbs. of ferro-silicon, assaying 83 per cent silicon and 0.28 per cent carbon, was fused in a Snyder electric furnace and there were added, in successive charges, 310 lbs. of chrome-iron ore, assay-ing 52.8 per cent chromium sesquioxide, together with 36 lbs. of lime and 28 lbs. of fluorspar. In this bath the silicon content, derived from the ferro-silicon, was equivalent to 162 lbs. sesquioxide of chromium, the chrome-iron ore employed representing 163 lbs. of chromium sesquioxide.

Assay of the metal on completion of the reduction gave:

|          | Per cent. |
|----------|-----------|
| Chromium | 67.00     |
| Silicon  | 6.04      |
| Carbon   | 0.13      |

To this initial metal there were added 3½ lbs. of ferro-manganese, containing 6 per cent of carbon and 76 per cent of manganese whereby 0.15 per cent of carbon and 1.9 per cent of manganese were introduced into the bath.

After complete fusion, this bath assayed approximately:

|           | Per cent. |
|-----------|-----------|
| Chromium  | 67.00     |
| Silicon   | 6.04      |
| Carbon    | 0.28      |
| Manganese | 1.90      |

An oxidizing blow was then passed through the molten mass for a period of two minutes, whereby there was obtained a final alloy assaying:

|           | Per cent. |
|-----------|-----------|
| Chromium  | 68.00     |
| Silicon   | 1.60      |
| Carbon    | 0.12      |
| Manganese | 0.30      |

*Example II.*

To a bath prepared by fusing 4 cwt. of steel scrap with 60 lbs. of chrome-iron ore, were added 63 lbs. of silico-manganese con-

taining 55 per cent of manganese and 25 per cent of silicon.

There was then introduced in successive charges a mixture of 200 lbs. of chrome-iron ore (52.8 per cent chromium sesquioxide) <sup>70</sup> and 50 lbs. of ferro-silicon (87 per cent silicon), followed by the addition of a further charge of 200 lbs. of the chrome-iron ore.

To assist the reaction the addition of a total of 40 lbs. of lime and 28 lbs. of fluorspar was made as required from time to time.

The reduced metal gave on analysis:

|           | Per cent. |
|-----------|-----------|
| Chromium  | 12.81     |
| Silicon   | 8.63      |
| Carbon    | 0.20      |
| Manganese | 5.83      |

The molten mass was then submitted to a blast of cold air, and prior to tapping, there were added to the blown metal 4 lbs. of ferro-manganese together with 4 ozs. of aluminium. The metal was run out into <sup>90</sup> the moulds and assayed:

|           | Per cent. |
|-----------|-----------|
| Chromium  | 13.59     |
| Silicon   | 0.23      |
| Carbon    | 0.12      |
| Manganese | 0.90      |

The yield of stainless metal so obtained was 3 cwt. 1 qr. 8 lbs.

The above examples are given for illustrative purposes and not by way of limitation, and it will be appreciated by those skilled in the art that the operative conditions, such, for instance, as the choice and proportions of the special reagents, will necessarily be adjusted according to the circumstances of any particular case, and the type of furnace available. These conditions may, however, be readily ascertained by a simple preliminary trial.

The use of a metal such as manganese has the effect of maintaining the thermal equilibrium necessary for satisfactory oxidation of the impurities in the initial alloy by the blow, and tends to provide a fluid slag as well as to impede the oxidation of the chromium. The presence of a certain quantity of manganese in ferro-chrome is also of advantage in that when the alloy is added to a bath of steel or iron the manganese assists deoxidation of the metal, and thereby tends to prevent any further loss of chromium through conversion into oxide. We have found that by operating according to this invention, the silicon and carbon impurities can be eliminated to within the limits of <sup>115</sup> analyses of commercial low-carbon and carbon-free ferro-chromium alloys without substantial loss of chromium due to oxidation.

It will be understood that the additional oxidizable element added to the ferro-chro-

mium alloy to impede the oxidation of the chromium during the blowing operation must not be one whose presence in the final purified metal will be detrimental to the latter in any particular application for which it is intended. Thus, if tungsten be said element, care must be observed in the case of an alloy of the composition of unstainable metal not to leave any material proportion of tungsten in the finished alloy as otherwise the deformable properties of the latter may be impaired.

It will be understood that the reduction of the chromite may be effected either in the presence of the bath of iron or separately therefrom, the invention not being limited in this respect.

I claim:

1. In the manufacture of an alloy of iron and chromium, the method of removing an impurity from a ferrous bath containing chromium consisting in submitting the bath to an oxidizing blow in the presence of manganese in such quantity that the chromium is protected from oxidation during the blowing operation.
2. In the manufacture of an alloy of iron and chromium, the method of removing impurities from a ferrous bath containing chromium consisting in submitting the bath to an oxidizing blow in the presence of manganese, the manganese present constituting not substantially less than 2% of the bath.
3. In the manufacture of an alloy of iron and chromium, the method of removing silicon existing as an impurity in a ferrous bath containing chromium, consisting in submitting the bath to an oxidizing blow in the presence of manganese to an amount not substantially less than 2% of the bath.
4. The process of manufacture of an unstainable iron-chromium alloy metal which comprises subjecting a molten crude alloy of these metals containing oxidizable impurities and of a chromium content between substantially 9-16 per cent to an oxidizing

blow in presence of manganese in quantity not initially below substantially 2.5 per cent.

5. The process of manufacture of an unstainable iron-chromium alloy metal which comprises subjecting a molten crude alloy of these metals containing oxidizable impurities and of a chromium content between substantially 9 to 16 per cent to an oxidizing blow in presence of an initial minimum quantity of manganese represented by approximately two-thirds of the proportion of the total oxidizable impurities present in said crude metal and not less than substantially 2.5 per cent of manganese.

6. The process of manufacture of an unstainable iron-chromium alloy metal which comprises preparing a low-carbon basis alloy of a chromium content between substantially 9 to 16 per cent by reducing a reducible chromium compound with a low-carbon silicon reducer within a ferrous bath, and subjecting the low-carbon basis alloy so produced to desilicizing with an oxidizing blow in presence of an initial minimum quantity of manganese represented by approximately two-thirds of the total oxidizable impurities present in said basis metal and not less than substantially 2.5 per cent of manganese.

7. The process of manufacture of an unstainable iron-chromium alloy metal which comprises preparing a low-carbon basis alloy by reducing chromite with a low-carbon silicon reducer within a ferrous bath proportioned to give a basis alloy containing between substantially 9-16 per cent of chromium, and then subjecting the low-carbon basis metal so produced to desilicizing with an oxidizing blow in presence of an initial minimum quantity of manganese represented by approximately two-thirds of the total oxidizable impurities present in said basis metal and not less than substantially 2.5 per cent of manganese.

In testimony whereof I have signed my name to this specification.

RONALD WILD.